

Patented Jan. 29, 1935

1,989,250

# UNITED STATES PATENT OFFICE

1,989,250

## OFFSET PRINTING INK

Charles P. Shaw, Detroit, Mich., assignor to  
Detroit Moulding Corporation, Detroit, Mich.

No Drawing. Application July 28, 1933,  
Serial No. 682,628

5 Claims. (Cl. 134—35)

The main objects of my invention are:

First, to provide an improved ink for offset printing and more especially for the offset printing of wood grain effects in relief.

Second, to provide a printing ink of this character, which is composed of commercially available offset printing ink and a thinner containing readily available ingredients.

Third, to provide offset printing ink of this character, which lays down perfectly on the printing plate yet which is not so thin as to fill up the half-tone plate.

Objects relating to details and economies of my invention will appear from the description to follow. The invention is defined and pointed out in the claims.

The printing plate is made planographic by the half-tone process with the design in relief. This is inked by a suitable machine or apparatus or by passing an ink roller over the plate, the ink not being forced down into the recesses, but remaining on the relief or high parts of the plate. A rubber or composition transfer roller is then run over the plate and the design transferred to the panel or object to be ornamented.

In this method of offset printing, with surface printing plates as distinguished from intaglio plates, especially with regard to decorating garnish moldings, the method of or agent for producing the offset printing ink is of prime importance. The thinner the ink with a sufficient color, the better the print. Thinned ink readily lifts from the plate and readily releases from the printing roll. The ink must lay down perfectly and yet not be so thin as to fill up the printing plate.

Oil added to the ink will allow it to release from the printing roll, but if used alone makes the ink too thin, fills up the plate and greatly cuts the color of the print. Greasy compounds aid in making the ink lay down and do not cut the color. However, a large amount of such compounds are required for satisfactory results, and further, there is a tendency for them to slur the printing.

I provide a thinner which combines the advantages of oil and greasy compounds, but which eliminates their disadvantages. I add to the offset printing ink a thinner containing the following ingredients by weight:

50 Castor oil 1.8 oz. 15.9%  
Colorless "00" Litho varnish 2.5 oz. 22.1%  
Stearine 3.0 oz. 26.6%  
Turpentine 4.0 oz. 35.4%

55 The castor oil, vanish, and stearine are dissolved in the turpentine and the ingredients are combined by the use of heat. Sufficient thinner is added to the offset printing ink until the latter is reduced to the proper consistency.

60 While any commercially available offset print-

ing ink may be used with my thinner, I prefer to use offset printing ink containing by weight pigment 35% to 40% and vehicle 65% to 60%. The pigment may be carbon black and the vehicle a heavy bodied linseed oil with a drier of the rosin type. Offset printing ink of this character may be readily bought or it may be duplicated by any ink manufacturer having facilities for grinding in pigments. In the case of black ink, the weight of the pigment is about 35% and the vehicle 65%. In the case of brown ink, the pigment runs up to 40% and the vehicle 60%. The vehicle itself is from 25% to 30% of the total weight, heavy bodied linseed oil, and 35% of the total weight, varnish.

Summarizing the analysis of the offset printing ink:

|             | Black   | Brown   | 20 |
|-------------|---------|---------|----|
|             | Percent | Percent |    |
| Linseed oil | 30      | 25      |    |
| Varnish     | 35      | 35      |    |
| Pigment     | 35      | 40      |    |

While the ratio of my thinner or reducing agent to the offset printing ink will vary with different printing conditions, nevertheless I prefer to use 14 parts by weight of my thinner to 86 parts by weight of the offset printing ink.

This preferred ratio of thinner to offset printing ink results in an ink which is of such character that a sufficient quantity thereof is held on the high point or design of the relief printing plate so that an effective transfer is made possible and that very good results are produced.

When the black ink is mixed according to the foregoing description, it comprises in composition by weight the ingredients as follows:

|                     | Per cent | Per cent | 40 |
|---------------------|----------|----------|----|
| Thinner             | 14       |          |    |
| Castor oil          | .14x15.9 | 2.2      |    |
| Varnish             | .14x22.1 | 3.1      |    |
| Stearine            | .14x26.6 | 3.7      |    |
| Turpentine          | .14x35.4 | 5.0      | 45 |
| Offset printing ink | 86       |          |    |
| Linseed oil         | .86x30   | 25.8     |    |
| Varnish             | .86x35   | 30.1     |    |
| Pigment             | .86x35   | 30.1     |    |
|                     |          |          | 50 |
| Total               | 100      | 100.0    |    |

The combined vanish content is thus 33.2% in the above composition.

In the brown ink, the pigment comprises 34.4% of the whole mixture, and the linseed oil 21.5%.

My ink is especially useful in the ornamenting of metal with imitation wood graining. The plate is prepared from a photograph by the half-tone process and with the graining design in relief.

The plate is inked with my special ink by passing an inking roller over the plate, the ink not being forced down into the recesses, but remaining on the relief or high parts of the printing plate. A pick-up or transfer roller is then run over the inked plate and the graining design transferred to the panel or surface to be ornamented.

The character of my special ink is such that it is held on the relief or high part of the plate without filling the same and readily releases from the transfer or printing roll and the plate. My thinner produces these advantages without cutting the color of the offset printing ink and without slurring the printing. These characteristics and advantages are highly desirable in the offset printing of delicate graining effects.

Having thus described my invention, what I claim as new and desire to secure by Letters Patent is:

20 1. An ink comprising in composition offset printing ink containing by weight: 25% linseed oil, 35% varnish, and 40% brown pigment; and a thinner containing by weight: 15.9% castor oil, 22.1% Colorless "00" Litho varnish, 26.6% stearine, and 35.4% turpentine; 14 parts by weight of thinner being added to 86 parts by weight of offset printing ink.

2. An ink comprising in composition offset printing ink containing by weight: 30% linseed oil, 35% varnish, and 35% black pigment; and a thinner containing by weight 15.9% castor oil, 22.1% Colorless "00" Litho varnish, 26.6% stearine, and 35.4% turpentine; 14 parts by weight of thinner being added to 86 parts by weight of offset printing ink.

3. An ink of the character set forth, comprising in composition offset printing ink containing by weight 35% to 40% pigment and 65% to 60% vehicle, the vehicle consisting of varnish and linseed oil, and a thinner or reducing agent containing by weight substantially 16% castor oil, 22% varnish, 27% stearine and 35% turpentine, substantially 14 parts by weight of the thinner or reducing agent being mixed with 86 parts by weight of the offset printing ink.

4. An ink of the character set forth, comprising in composition by weight substantially: 30.1% pigment, 25.8% linseed oil, 33.2% varnish, 2.2% castor oil, 3.7% stearine, and 5.0% turpentine.

5. An ink of the character set forth, comprising in composition by weight substantially: 34.4% pigment, 21.5% linseed oil, 33.2% varnish, 2.2% castor oil, 3.7% stearine, and 5.0% turpentine.

CHARLES P. SHAW.